# EUROPEAN PATENT SPECIFICATION

(11) **EP 0 524 155 B1**
(45) Date of publication and mention of the grant of the patent: **23.12.1998**
(21) Application number: 92830278.5
(22) Date of filing: 28.05.1992
(51) Int. Cl.: B05D 7/16, B05D 5/08, B05D 7/00

(54) **Industrial procedure for the application of a P.T.F.E. film on aluminium surfaces**
Industrielles Verfahren zum Aufbringen eines P.T.F.E.-Films auf Aluminium-Oberflächen
Procédure industrielle pour l'application d'un film P.T.F.E. sur des surfaces en aluminium

(30) Priority: 04.07.1991 IT AN910025
(43) Date of publication of application: 20.01.1993
(73) Proprietor: ALLUFLON S.p.A., I-61040 Mondavio (PS) (IT)
(72) Inventor: Montagna, Michele, I-61100 Pesaro (IT)
(74) Representative: Baldi, Claudio

(56) References cited:
- WO-A-91/02773
- US-A- 4 177 320

## Description

This patent application concerns an industrial procedure for the application of a polytetrafluoroethylene film on aluminium surfaces by means of mechanical-chemical bonding using a specific compound.

In order to understand and appreciate the characteristics and advantages of the procedure according to the invention, some mention must be made of the technology used to date for covering metal surfaces with P.T.F.E. (polytetrafluoroethylene) film, which is more commonly known under its commercial name of "TEFLON".

P.T.F.E. is an organic compound which can continuously resist temperatures of up to 250°C or temperatures of up to 400°C for shorter periods of time.

This property, together with its excellent non-adhering qualities has resulted in its extensive use in the production of cooking pots and pans and crockery used in the home and for all those articles which require easy cleaning and resistance to high temperatures.

If on one hand the non-adhering quality of this organic compound makes the items on which it is used easy to clean, on the other hand, this very quality creates the problem of how to adhere the P.T.F.E. to the surfaces treated, since P.T.F.E. is very difficult to bond chemically to all other materials, in particular with aluminium, glass or ceramics, which are the materials principally used for manufacturing kitchenware.

Despite this, it has been proved that it is possible to adhere P.T.F.E. to an aluminium surface if the latter is roughened so as to provide a mechanical hold for the film of P.T.F.E.

One of the most common and widely used methods for roughening this material consists of chemical pickling which attacks the metal surface which is to be coated, with NaOH (sodium hydroxide, commonly known as caustic soda) and HCl (hydrochloric acid).

In the production of aluminium pots and pans, the metal disks, in various diameters and thickness, are dipped in a bath of NaOH to be degreased and then in successive baths of HCl which attacks the metal surface thereby making it rough, and covering the same with micro-cavities so that it provides the required mechanical hold.

P.T.F.E. is sprayed on the surface of the disk in an aqueous solution to ensure its penetration in the pores produced by the previous pickling treatment; the disk is then placed in kilns, where the P.T.F.E. is sintered at a temperature of 370°C; once the P.T.F.E. has solidified it is trapped in the micro-cavities on the metal surface.

The above system is commonly used in the manufacture of pots and pans; the system used consists of a pickling procedure whereby the disks are first placed into treatment tanks and are then rinsed and dried and then transported to a series of "rolling machines" which apply the layer of P.T.F.E. with a lithographic type technique.

Each rolling machine consists of two rollers, one of which is in metal and the other in rubber, which rotate touching each other, with the aqueous solution of P.T.F.E. running over them; the bottom side of the rubber roller touches the pickled disks and uniformly distributes the P.T.F.E. solution on the same.

In order to increase the thickness of the layer of P.T.F.E. coating, a set of rolling machines is used by means of which the disk receives successive coats of the product, between which it is dried; in general, there are four rolling machines on each of which is applied the aqueous solution of P.T.F.E. with the addition of pigments.

The above procedure consists of a thorough pickling of the aluminium which causes large quantities of metal to be removed and which remain bound to the acids and the bases of the baths, very quickly depleting their corrosive properties.

The solution in the tank must therefore be replaced very frequently and the depleted solution must be processed through purifying systems before being drained in the sewage system.

In view of the fact that water and mud containing aluminium salts in an amount directly proportional to the amount of aluminium in the solution are obtained from the purification of depleted solutions, the discharge of the these muds in the sewage system increases the overall management costs of the purification system, which in itself is very high.

The purpose of this invention is to design a new industrial process for coating aluminium surfaces with P.T.F.E. more quickly, cheaply and with less pollution with respect to the above, thanks to the fact that no deep pickling treatment is required for roughening the surface.

The procedure according to the invention involves the coating on a previous degreased metal surface of a product (P), on one hand adhering to a smooth aluminium surface and on the other permitting the formation of a mechanical-chemical bonding with the P.T.F.E.

This new industrial procedure consists of the following phases: the metal surface is degreased with NaOH (sodium hydroxide) which removes all oxides and/or grease, which would compromise the efficiency of the successive treatments; it should be remembered that aluminium is chemically reactive to soda, so that the surface of the disk is attacked to some extent during this initial phase of production.

After treatment in NaOH (sodium hydroxide), the aluminium disks are washed in water and conveyed directly to the drying phase which is followed by a "rolling" process by means of a set of four rolling machines, the first two of which spread the above product (P) on the aluminium disks; said product (P) binds to the smooth metal surface with a mechanical-chemical action, consequently becoming the anchoring surface for the external P.T.F.E. coating.

After the initial degreasing phase, it is recommended, but not absolutely necessary, to place the parts very briefly in an acid bath (10-12 seconds) in order to remove any soda residues which might damage the system.

The product (P) which has this functional bivalence is obtained by mixing a polyamide-imide resin (know on the market as RHODEFTAL 200) with dimethylaminoethanol (commercial name REXOLIN) and water in the following percentages:

| | |
|---|---|
| A - RHODEFTAL 200 (Polyamide-imide) | 35.714% by weight |
| B - REXOLIN (dimethylaminoethanol) | 7.143% by weight |
| C - WATER | 57.143% by weight |

The mixture percentage of component (A) with respect to component (B) may vary by plus or minus 5% by weight, as may do the mixture percentage of component (C) with respect to the sum of the components (B+C).

According to the procedure in question, in the first rolling machine, this product (P) is used mixed with a thickening solution and colouring pigments, while in the second rolling machine the P.T.F.E. is added to the mixture used on the first rolling machine; in the last two rolling machines, an aqueous solution of P.T.F.E. is used with the additions of pigments.

The mixture used in the first rolling machine consists of the following components in the following percentages:

| | |
|---|---|
| - Product (P) | 80% by weight |
| - thickening solution + colouring pigments | 20% by weight |

wherein the composition of the product (P) with respect to the thickening solution may vary by plus or minus 0.5% and wherein the percentage of pigments in the thickening solution may vary from 8% - 12% by weight.

The mixture used in the second rolling machine consists of the following components in the following percentages:

| | |
|---|---|
| - Product (P) | 50% by weight |
| - P.T.F.E. (commercial name HOSTAFLON) | 25% by weight |
| - thickening solution + colouring pigments | 25% by weight |

wherein the composition of the product (P) with respect to the sum of the other two components may vary by plus or minus 5% by weight and wherein the percentage of pigments in the thickening solution may vary from 8% - 12% by weight.

The mixture used in the third and fourth roller is a standard aqueous solution of P.T.F.E. and colouring pigments.

The thickening solution in the mixture used in the first and in the second rolling machine consists of the following components in the following percentages:

| | |
|---|---|
| D - ISOBUTYL alcohol | 11.4% by weight |
| E - SOLVENT S11 (dichloropropane hexane) | 9,5% by weight |
| F - EMPILAN NP9 (alkylphenolethoxylate) | 79.1% by weight |

The mixture percentage of the component (F) with respect to the sum of the components (D+E) may vary by plus or minus 8%.

Considering the above, the advantages offered by the procedure according to the invention are now more appreciable.

In preparing the metal surface it is not necessary to attack the same in depth and therefore the disks do not need to be dipped in solutions but simply sprayed with solutions as in the case of standard wash tunnels.

If, for reasons of the investment, the former dipping system is to be continued, there will still be a reduction in management costs and times; in fact the system processing times are significantly reduced (from the current twenty minutes to three minutes with the procedure according to the invention), while the solutions used in this new procedure can treat major surface areas thereby reducing the purchasing costs of the solution and of the costs for treating depleted solutions and the muds produced.

On the whole, the entire process for application of the P.T.F.E. film is faster in that the times required for preparing the aluminium surfaces are lower.

## Claims

1. An industrial procedure for the application of P.T.F.E. film on aluminium surfaces consisting of the following sequence of production phases:
a) degreasing with sodium hydroxide in an aqueous solution;
b) washing with water;
c) an optional rapid bath (10-12 seconds) in a hydrochloric acid solution followed by rinsing in water;
d) drying;
e) a rolling process through a set of four rolling machines in which:
I) the mixture used in the first rolling machine consists of:
| | |
|---|---|
| - Product (P) | 80% by weight |
| - thickening solution + colouring pigments | 20% by weight |
wherehin the composition of the product (P) with respect to the thickening solution may vary by plus or minus 0.5% and wherein the percentage of pigments in the thickening solution may vary from 8% - 12% by weight.
II) the mixture used in the second rolling machine consists of:
| | |
|---|---|
| - Product (P) | 50% by weight |
| - P.T.F.E. (commercial name HOSTAFLON) | 25% by weight |
| - thickening solution + colouring pigments | 25% by weight |
wherein the composition of the product (P) with respect to the sum of the other two components may vary by plus or minus 5% by weight and wherein the percentage of pigments in the thickening solution may vary from 8% - 12% by weight.
III) the mixture used in the third and fourth rolling machines is a standard aqueous solution of P.T.F.E. and colouring pigments;
wherein the above product (P) consists of:
| | |
|---|---|
| A) RHODEFTAL 200 (Polyamide-imide) | 35.714% by weight |
| B) REXOLIN (dimethylaminoethanol) | 7.143% by weight |
| C) WATER | 57.143% by weight |
wherein the thickening solution in the mixture used in the first and second rolling machines consists of the following components in the following percentages:
| | |
|---|---|
| D) ISOBUTYL alcohol | 11.4% by weight |
| E) SOLVENT S11 (dichloropropane/hexane) | 9.5% by weight |
| F) EMPILAN NP9 (alkylphenolethoxylate) | 79.1% by weight |
and wherein in product (P) the mixture percentage of the component (A) with respect to component (B) may vary by plus or minus 5% by weight, as may the mixture percentage of the component (C) with respect to the sum of components (A+B).

2. An industrial procedure for the application of P.T.F.E. film on aluminium surfaces according to claim 1) characterized in that in product (P) the mixture percentage of the component (A) with respect to component (B) may vary by plus or minus 5%, as may the mixture percentage of the component (C) with respect to the sum of components (A+B).

3. An industrial procedure for the application of P.T.F.E. film on aluminium surfaces according to claim 1) characterized in that in the mixture used in the first rolling machine the composition of the product (P) with respect to the thickening solution may vary by plus or minus 0.5% and that the percentage of pigments in the thickening solution may vary from 8% - 12%.

4. An industrial procedure for the application of P.T.F.E. film on aluminium surfaces according to claim 1) characterized in that in the mixture used in the second rolling machine the composition of the product (P) with respect to the sum of the other two components may vary by plus or minus 5% and that the percentage of pigments in the thickening solution may vary from 8% - 12%.

## Patentansprüche

1. Industrielles Verfahren zum Aufbringen von P.T.F.E.-Folie auf Aluminiumflächen, dadurch gekennzeichnet, daß dieses Verfahren folgende Arbeitsschritte umfaßt:
a) Entfettung mittels Natriumhydroxid in wässriger Lösung;
b) Reinigung mit Wasser;
c) Eventuelles Tauchbad (10 - 12 Sekunden) in einer Salzsäurelösung und anschließendes Spülen in Wasser;
d) Trocknen
e) Walzvorgang mittels einer aus vier Walzen bestehenden Anlage, wobei
I. die auf der ersten Walze verwendete Mischung wie folgt zusammengesetzt ist:
| | |
|---|---|
| - Produkt (P) | 80 Gewichts% |
| - Eindickungsmittel + Farbstoffe | 20 Gewichts%, |
wobei die Zusammensetzung des Produkts (P) bezogen auf das Eindickungsmittel um 0,5 Gewichts% nach oben oder unten schwanken und der Prozentsatz der im Eindickungsmittel enthaltenen Farbstoffe zwischen 8 und 12 Gewichts% abweichen kann;
II. die auf der zweiten Walze verwendete Mischung wie folgt zusammengesetzt ist:
| | |
|---|---|
| - Produkt (P) | 50 Gewichts% |
| - P.T.F.E. (Handelsname HOSTFLON) | 25 Gewichts% |
| - Eindickungsmittel + Farbstoffe | 25 Gewichts%, |
wobei die Zusammensetzung des Produkts (P) bezogen auf die übrigen beiden Bestandteile um 5 Gewichts% nach oben oder unten schwanken und der Prozentsatz der im Eindickungsmittel enthaltenen Farbstoffe zwischen 8 und 12 Gewichts% abweichen kann;
III. die auf der dritten und vierten Walze verwendete Mischung eine Dispersion von P.T.F.E. und Farbstoffen in Wasser darstellt; wobei vorgesehen ist, daß das besagte Produkt (P) wie folgt zusammengesetzt ist:
| | |
|---|---|
| A) RHODEFTAL 200 (Polyamid-Imid) | 35,714 Gewichts% |
| B) REXOLIN (Dimethylaminäthanol) | 7,143 Gewichts% |
| C) WASSER | 57,143 Gewichts%, |
wobei vorsehen ist, daß das auf der ersten und der zweiten Walze verwendete Eindickungsmittel aus folgenden Bestandteilen in den jeweils genannten Prozentsätzen besteht:
| | |
|---|---|
| D) Isobuthyl-ALKOHOL | 11,4 Gewichts% |
| E) LÖSUNGSMITTEL S11 (Dichlorpropanhexan) | 9,5 Gewichts% |
| F) EMPILAN NP9 (Alkylphenoläthoxylat) | 79,1 Gewichts%, |
wobei außerdem vorgesehen ist, daß der im Produkt (P) enthaltene Prozentsatz des Bestandteils (A) bezogen auf Bestandteil (B) um 5 Gewichts% nach oben oder unten schwanken kann. Dies gilt im gleichen Maß auch für den Prozentsatz des Bestandteils (C) bezogen auf die Summe der Bestandteile (A+B).

2. Industrielles Verfahren zum Aufbringen von P.T.F.E.-Folie auf Aluminiumflächen gemäß Anspruch 1, dadurch gekennzeichnet, daß der Prozentsatz des im Produkt (P) enthaltenen Bestandteils (A) bezogen auf Bestandteil (B) ebenso wie der Prozentsatz des Bestandteils (C) bezogen auf die Summe der Bestandteile (A+B) um 5% nach oben oder unten schwanken kann.

3. Industrielles Verfahren zum Aufbringen von P.T.F.E.-Folie auf Aluminiumflächen gemäß Anspruch 1, dadurch gekennzeichnet, daß die Zusammensetzung des auf der ersten Walze verwendeten Produkts (P) bezogen auf das Eindickungsmittel um 0,5 % und der Prozentsatz der Farbstoffe im Eindickungsmittel zwischen 8% und 12% nach oben oder unten schwanken kann.

4. Industrielles Verfahren zum Aufbringen von P.T.F.E.-Folie auf Aluminiumflächen gemäß Anspruch 1, dadurch gekennzeichnet, daß die Zusammensetzung des auf der zweiten Walze verwendeten Produkts (P) bezogen auf die Summe der übrigen beiden Bestandteile um 5% nach oben oder unten schwanken und der Prozentsatz der Farbstoffe im Eindickungsmittel zwischen 8% und 12% abweichen kann.

## Revendications

1. Processus industriel pour l'application d'une pellicule de P.T.F.E. sur des surfaces en aluminium, caractérisé en ce qu'il comprend la suivante séquence de phases opérationnelles: a) traitement de dégraissage à l'aide d'hydroxyde de sodium en solution aqueuse;
b) lavage à l'eau;
c) éventuel bain rapide (10-12 secondes) dans solution d'acide chlorhydrique et successif rinçage dans l'eau;
d) séchage;
e) processus de laminage par le biais d'une batterie de quatre laminoirs et où:
I°) le mélange utilisé dans le premier laminoir est composé de:
| | |
|---|---|
| - Produit (P) | 80% en poids |
| - Solution épaississante+pigments | colorants 20% en poids |
où la composition du produit (P), par rapport à la solution épaississante, peut varier de plus ou moins 0,5% en poids et où le pourcentage de pigments présents dans la solution épaississante peut varier du 8% au 12% en poids.
II°) le mélange utilisé dans le deuxième laminoir est composé de:
| | |
|---|---|
| - Produit (P) | 50% en poids |
| - P.T.F.E. (nom commercial HOSTAFLON) | 25% en poids |
| - Solution épaississante+pigments colorants | 25% en poids |
où la composition du produit (P), par rapport à la somme des deux autres composants, peut varier de plus ou moins 5% en poids et où le pourcentage de pigments présents dans la solution épaississante peut varier du 8% au 12% en poids.
III°) le mélange utilisé dans le troisième et le quatrième laminoir est une usuelle dispersion aqueuse de P.T.F.E. et de pigments colorants; étant prévu que le précité produit (P) soit composé de:
| | |
|---|---|
| A) RHODEFTAL 200 (Polyamide-imide) | 35,714% en poids |
| B) REXOLYN (diméthylamino-éthanol) | 7,143% en poids |
| C) EAU | 57,143% en poids |
étant prévu que la solution épaississante présente dans le mélange utilisé dans le premier et dans le deuxième laminoir soit formée des composants suivants, dans les pourcentages suivants:
| | |
|---|---|
| D) ALCOOL Isobutylique | 11,4% en poids |
| E) SOLVANT S11 (Hexane dichloropropane) | 9,5% en poids |
| F) EMPILAN NP9 (Alkylphénoléthyloxylate) | 79,1% en poids |
étant également prévu que dans le produit (P), le pourcentage du mélange du composant (A) par rapport au composant (B) peut varier de plus ou moins 5% en poids, et de même en ce qui concerne le pourcentage de mélange du composant (C) par rapport à la somme des composants (A+B).

2. Processus industriel pour l'application d'une pellicule de P.T.F.E. sur des surfaces en aluminium, selon la revendication 1, caractérisé en ce que dans le produit (P), le pourcentage de mélange du composant (A) par rapport au composant (B) peut varier de plus ou moins 5%, et de même en ce qui concerne le pourcentage de mélange du composant (C) par rapport à la somme des composants (A+B).

3. Processus industriel pour l'application d'une pellicule de P.T.F.E. sur des surfaces en aluminium, selon la revendication 1, caractérisé en ce que dans le mélange utilisé dans le premier laminoir, la composition du produit (P) par rapport à la solution épaississante peut varier de plus ou moins 0,5% et pour le fait que le pourcentage de pigments dans la solution épaississante peut varier du 8% au 12%.

4. Processus industriel pour l'application d'une pellicule de P.T.F.E. sur des surfaces en aluminium, selon la revendication 1, caractérisé en ce que dans le mélange utilisé dans le deuxième laminoir, la composition du produit (P) par rapport à la somme des deux autres composants peut varier de plus ou moins 5% et pour le fait que le pourcentage de pigments dans la solution épaississante peut varier du 8% au 12%.
